

F. VON WURSTEMBERGER.  
PROCESS FOR THE PROTECTION AGAINST ELECTROLYTIC DESTRUCTION.  
APPLICATION FILED JULY 23, 1920.

1,379,582.

Patented May 24, 1921.

Fig.1



Fig.2.



Inventor:

Franz von Wurstemberger,  
By Henry Orth

Atty.

# UNITED STATES PATENT OFFICE.

FRANZ VON WURSTEMBERGER, OF ZURICH, SWITZERLAND.

## PROCESS FOR THE PROTECTION AGAINST ELECTROLYTIC DESTRUCTION.

1,379,582.

Specification of Letters Patent. Patented May 24, 1921.

Application filed July 23, 1920. Serial No. 398,385.

To all whom it may concern:

Be it known that I, FRANZ VON WURSTEMBERGER, a citizen of the Republic of Switzerland, residing at Zurich, Hardturmstrasse 5 19, Switzerland, have invented certain new and useful Improvements in Processes for Protecting Against Electrolytic Destruction; and I do hereby declare the following to be a clear, full, and exact description of 10 the invention, such as will enable others skilled in the art to which it appertains to make and use the same, reference being had to the accompanying drawing, and to letters or figures of reference marked thereon, 15 which form a part of this specification.

The object of the present invention is a process for the protection against electrolytic destruction of certain parts of apparatus which contain at least two liquid- 20 spaces and are constructed of different metals.

It has been ascertained that certain cor- 25 rosions in the interior of tubes of heat ex- changing apparatus, condensers etc. and generally of parts which are in contact with 30 one of the liquid mediums, are the result of galvanic currents of low voltage, which are generated by the difference of potential, occurring in the space of the liquid medium between the exterior surface of the tube and the surface of wet parts of iron.

Such differences of potential are unavoid- 35 able when different metals are used in the construction of such an apparatus. The cur- rents generated in this way are very injuri- 40 ous to the metallic parts, if they have an opportunity to find their way into an ex- tended system of electrodes such as a heat exchange apparatus consisting of a quantity 45 of tubes. In consequence of polarization and depolarization, the different parts of such electrodes are unequally exposed to the electrolytic attack, so that the whole de- structive effect may be concentrated at cer- 50 tain spots and be the cause of their rapid destruction.

Referring to the drawings—

Figure 1 is a partial section of a condenser illustrating the corrosion currents. 55

Fig. 2 is a similar section showing one method of short-circuiting these currents.

Fig. 1 serves to explain these conditions for instance in the case of an ordinary condensing plant. The tubes of brass 1 (of 55 which only one is shown) are packed with rubber joints 2 in tube plates of brass (3)

which are riveted to the iron shell 4 of the condenser 5. 6 is a supporting plate of iron in the interior of the condenser.

The steam space is to be considered also 60 as a space containing liquid because the steam is to be condensed therein. Assuming that the condensed steam may contain impurities, such as a small quantity of salt, it will therefore be electrically conducting. 65 The point of contact 7 between tube and supporting plate is not a metal to metal one, because the supporting plate and its holes will soon be covered with a layer of rust which prevents a metallic contact and pos- 70 sses an electric conductivity only as carrier of an electrolyte. The tube or tubes on one hand, the supporting plate and shell on the other form in this way the electrodes of a galvanic cell. The path of the current 75 will be that shown in Fig. 1 by a dash and dot line provided with arrows. The nest of tubes will be anodic relative to the circulating water in space 10 and is subjected to 80 corrosions for this reason.

Protectors of zinc and iron used heretofore preserve the tubes from the harmful effect of such currents, by concentrating the destructive electrolytic action on the protectors themselves. The protecting effect is 85 usually incomplete.

With the new process which is the object of the present invention a much more effective protection is obtained by equalizing differences of potential which occur between 90 parts of different metals at their contact with a liquid acting as an electrolyte, by means of well conducting, durable short-circuits between these metallic parts themselves which act as electrodes. In this way the 95 wandering of currents into other circuits for instance such formed by liquids in other spaces and their respective metallic parts is prevented as well as any resulting electrolytic destruction of said parts. Galvanic 100 electrical corrosions on the less precious metal itself in the first space are of course not eliminated, they occur in the highest degree there where the two different metals are nearest to one another therefore at the 105 joints and the points of contact of the short circuits. They may be taken up by removable parts placed there to strengthen the exposed parts of the less precious metal.

In Fig. 2 an exemplification for carrying 110 out the process according to the invention on a condenser is illustrated. The joint be-

tween the two different metals is removed from 20 to 21 by choosing brass for the supporting plate instead of iron. The thick line 21 denotes a short-circuit joint made by 5 soldering. Instead of the direct soldering of the joint a connection soldered to both metals may be adopted. 22 is a strengthening ring which serves to take up the electrolytic attack. 23 is a well conducting 10 short-circuit joint between the latter and the end cover 26. This joint being outside of the waterspace a screw joint is sufficient for a durable connection. The currents which will occur will follow the circular 15 path indicated in chain-dotted lines. All other parts of iron or brass, especially the tubes are free from currents.

Different kinds of short circuiting devices have already been proposed, but the fact 20 that certain kinds of corosions of the more electro-positive metal in one liquid space were of electrolytic nature and were caused by currents which had their origin in another liquid space of the apparatus, was not 25 discovered. Under these conditions the proper adaption of short circuit devices was impossible. It was considered sufficient to exclude metallic parts for which a protection was required from a supposed path of 30 current, without considering where the currents were generated, while according to the present process such currents are collected

immediately at their point of origin and rendered harmless through shortcircuiting same. The meaning of "more electro-positive" is used in the same sense that copper 35 is more electro-positive than zinc and iron.

I claim:

1. The method of protecting from electrolytic destruction certain parts of apparatus which contain at least two liquid spaces and are constructed of different metals, from electrolytic destruction, which comprises equalizing the differences of potential that occur between any parts of different metals 45 contacting with a liquid acting as an electrolyte by connecting together those parts by well conducting durable short circuit devices.

2. The method of protecting from electrolytic destruction certain parts of apparatus which contain at least two liquid spaces and are constructed of different metals, which comprises equalizing the differences of potential that occur between any parts of different metals contacting with a liquid acting as an electrolyte by connecting together those parts by well conducting durable short circuit devices and providing removable strengthening elements of the less electro-positive metal on its most exposed places. 55

In testimony that I claim the foregoing as my invention, I have signed my name.

FRANZ VON WURSTEMBERGER.